

## UNITED STATES PATENT OFFICE.

MASAAKI YONEZU, OF TOKYO FU, AND EIICHIRO ENDO, OF TOKYO, JAPAN.

## COMPOSITION OF STAINLESS IRON ALLOY.

No Drawing.

Application filed April 23, 1924. Serial No. 708,566.

This invention relates to a composition of a stainless iron alloy consisting in adding to chromium steel from 1 to 10% of vanadium, and the object thereof is to change the physical properties of various kinds of high chromium steel and make them soft and malleable.

Various kinds of high chromium steel, say those containing from 8 to 30% of chromium have all of them the following properties:

1. A property to be hardened even in the air, that is if a high chromium steel is heated to red heat and allowed to cool in the air, without suddenly cooling it in water or oil, it becomes hardened.

Of course this property differs in degree according to kinds of such steel. For instance, in chromium steel having greater percentage of chromium or somewhat greater percentage of nickel, this property is not so conspicuous;

2. A high hardness, even if a high chromium steel is thoroughly annealed, it cannot be made as soft as annealed common carbon steel. Consequently, the work to be done in red heat is more difficult with it than with common carbon steel;

3. Difficulty in the work of scraping it or turning it in a lathe. If a high chromium steel thoroughly annealed is scraped or turned in a lathe, the cutting tool harder than the chromium steel soon becomes worn and broken at its edge, and

4. Difficulty of bending in the atmospheric temperature. If you bend high chromium steel at atmospheric temperature, it will become broken or cracked. Even if it is thoroughly annealed, it can only be bent to a slight curvature.

Common high chromium steel having such properties cannot be made into ornamental articles of delicate workmanship. It is also impossible to draw such steel into fine wire or roll same into thin sheets. But if a suitable percentage of vanadium is added to it, it will

1. Lose its property of becoming hardened, not only in the air but even if it is subjected to an ordinary hardening process, such as heating the metal to 1000° C. or more and suddenly cooling same in water, it will not become hardened. Consequently, there is no need of annealing such steel.

2. Become soft, high chromium steel un-annealed but containing vanadium being softer than high chromium steel containing no vanadium but annealed, thus decreasing the difficulty of the work of scraping, turning in a lathe, and working the steel heated, and

3. Become flexible at atmospheric temperatures, high chromium steel unannealed but containing vanadium being far more flexible than high chromium steel annealed but containing no vanadium.

It may here be noted that the softness and the property of flexibility are not, evidently, the result of the steel losing its property of becoming hardened.

The above properties are not apparent if the proportion of vanadium is less than 1%, but become apparent gradually as the proportion increases, and being most evident when the proportion of vanadium is 4 or 5%.

Moreover, the properties do not become stronger even if the proportion of vanadium is increased, but on the contrary too much vanadium has injurious effects on the alloy. Consequently the proportion of vanadium should not exceed 10%. Of course the effects of the addition of vanadium are different for different kinds of steel, but for example an alloy whose composition is Cr. 13%, V. 4% and C. O. 3%, the remainder being iron, the hardness has been found to be 130 by Brinell test of hardness, it being the same whether the alloy is subjected to hardening or to annealing processes, and as to flexibility, the steel can be bent 180° without cracks.

The effects of carbon on the physical properties of steel is stronger and more apparent in high chromium steel than in common carbon steel, but if a suitable proportion of vanadium is added thereto, the quantity of carbon contained has no effect on the physical properties of the alloy.

The following is an example of carrying my invention into effect:

Melt iron in a furnace and add thereto chromium, or ferro-chromium previously measured. When the two have become perfectly fused, add thereto a suitable quantity of ferro-vanadium. Vanadium in the molten state oxidizes quickly and floats in the molten mass. Therefore the molten mass in the

furnace must be poured quickly into a mold percent of chromium and 1 to 10 percent of as soon as it attains a suitable degree of vanadium, the remainder being iron.

In this invention, there is no harm in adding nickel or any metal besides vanadium.

We claim:

A stainless iron alloy consisting of 8 to 30

In testimony whereof we have signed our names to this specification. 10

MASAAKI YONEZU.  
EITARO ENDO.